

April 9, 1946.

R. C. HOUCK ET AL

2,398,004

CONTROLLING THE ISOELECTRIC POINT OF GELATIN

Filed July 20, 1943



ROBERT C. HOUCK  
JOHN RUSSELL  
SAMUEL E. SHEPPARD  
INVENTORS

BY *Newton M. Perrine*  
*R. Frank Smith*  
ATTORNEYS

## UNITED STATES PATENT OFFICE

2,398,004

CONTROLLING THE ISOELECTRIC POINT  
OF GELATIN

Robert C. Houck, John Russell, and Samuel E. Sheppard, Rochester, N. Y., assignors to Eastman Kodak Company, Rochester, N. Y., a corporation of New Jersey

Application July 20, 1943, Serial No. 495,454

6 Claims. (Cl. 260—118)

This invention relates to the manufacture of gelatin and particularly to a method for controlling the isoelectric point of gelatin.

It is known that the properties of gelatin can be changed markedly by the method of manufacture of the gelatin. Such properties include viscosity, swelling, dyeing, alcohol precipitation and isoelectric point. With respect to these properties, the isoelectric point is a critical point. Control of the isoelectric point permits control of the variation of these properties, this being important for gelatin used in making photographic emulsions and in gelatins used in wash-off relief and inbibition photographic color processes.

The isoelectric point of a material is the pH value at which it is electrically neutral when in solution. For an amphoteric substance such as gelatin, the isoelectric point is the pH at which it is equally dissociated as an acid and as a base. The isoelectric point of gelatin depends upon the method by which the gelatin has been made. Gelatins made by the lime process of plumping of hides have an isoelectric point of from 4.7 to 5.0 and their physical properties usually exhibit a sharp minimum somewhere in this region. Gelatins extracted by the acid process have an isoelectric point varying from pH 7 to pH 9 and their physical properties usually do not exhibit a sharp minimum but a flat region as shown, for example, in Sheppard and Hudson U. S. Patent 2,101,877, granted December 14, 1937.

It is desirable in certain processes to have a gelatin having an isoelectric point below the values usually obtained when the material is extracted by the acid process. The pH of the isoelectric point of the gelatin is not readily controlled by varying the method of extraction from the hides and the gelatin obtained does not always have an isoelectric point in the desired region.

It is, therefore, an object of the present invention to provide a method for controlling the isoelectric point of gelatin. A further object is to provide a method for obtaining gelatin of any desired isoelectric point. A still further object is to provide a method for lowering the isoelectric point of gelatin and thereby controlling its physical properties such as swelling and viscosity. Other objects will appear from the following description of our invention.

These objects are accomplished by heating gelatin in the presence of any material which raises the pH of the gelatin solution, such as an alkaline hydroxide, for a definite period of time and

then stopping the action of the alkali and washing it from the gelatin.

The accompanying drawing shows a series of graphs illustrating the change in isoelectric point obtained by treating an acid process gelatin for varying periods of time at various degrees of alkalinity.

Our method consists in treating gelatin, preferably gelatin of high isoelectric point, with any material which raises the pH of the solution, such as an alkali metal hydroxide, an alkaline earth metal hydroxide, an alkali carbonate, triethanolamine, or pyridine for a definite period of time. The time required depends upon the temperature and the pH at which the gelatin is heated or aged. The speed of the drop in isoelectric point at a given pH is affected by the temperature which can be varied from 5° C. to 60° C. The pH can be varied from 8 to 12.5, the rate change at a given temperature increasing with increase in pH from 8 to 12.5. At the end of the desired time, the action of the alkali is stopped by adding acid to neutralize the alkali. The resulting gelatin is chilled, noodled and washed. It will then have an isoelectric point which depends upon the time, temperature and pH of treatment as stated above.

According to our method a solution of gelatin is made in the usual manner and the desired amount of an aqueous solution of an alkaline material, such as alkali metal hydroxide or alkaline earth metal hydroxide added to it to bring the pH to the desired point as explained below. The solution is then heated for a definite period of time and at the end of this time the reaction is stopped by adding sufficient acid such as hydrochloric acid to neutralize the alkali which was added to the gelatin. The resulting gelatin is then chilled, noodled and washed for about 48 hours with cold distilled water.

We have treated both acid-process gelatin and lime-process gelatin by our method but find it preferable to treat the acid-process gelatin. Results obtained by treating the various types of gelatin were ascertained by determining the isoelectric point by the turbidity method or the cataphoresis method at 25° C. The turbidity method was described by Sheppard and Houck in an article published in Journal of Physical Chemistry, Vol. 34, 1930, page 2187. The effect on acid-process gelatin of variations in pH, time of heating and temperature of treatment were determined and are given in the following tables.

The effect of pH on the isoelectric point of an acid-process gelatin treated at 52° C. for various lengths of time is recorded in the following table.

Gelatin having originally an isoelectric point at pH 9.17 was mixed with a sufficient quantity of sodium hydroxide solution to bring the pH to the value noted at the top of the table, that is, pH 8, pH 9.6, etc. The pH of the isoelectric point should not be confused with the pH of treatment. Although the gelatin had an isoelectric point at pH 9.17, the pH of the solution of the gelatin in water was about 7 and it was necessary to add an alkali to the gelatin to bring the pH to 8 and the higher values at which portions of the gelatin were treated. The results of this treatment were as follows:

| Time of treatment<br>(hours) | pH of isoelectric point |        |         |         |
|------------------------------|-------------------------|--------|---------|---------|
|                              | pH 8                    | pH 9.6 | pH 10.6 | pH 12.2 |
| 0.0                          | 9.17                    | 9.17   | 9.17    | 9.17    |
| .016 (1 min.)                |                         |        |         | 7.16    |
| .16 (10 min.)                |                         |        |         | 6.43    |
| .33 (20 min.)                |                         |        |         | 5.90    |
| .66 (40 min.)                |                         |        |         |         |
| 1.0                          |                         |        | 7.64    | 5.15    |
| 1.5                          |                         |        |         | 4.98    |
| 2.0                          | 9.12                    | 8.88   | 7.04    |         |
| 3.5                          |                         |        |         | 4.5     |
| 4.0                          | 89.96                   |        |         |         |
| 5.0                          |                         | 7.82   | 6.46    |         |
| 24.0                         | 8.56                    |        |         |         |
| 28.0                         |                         | 6.08   | 5.4     |         |
| 50.0                         | 6.54                    | 4.91   | 4.8     |         |

These data were plotted as shown in the accompanying drawing to indicate the change in pH of the isoelectric point for various times of treatment. A study of the table and the curves shows that the decrease in isoelectric point is regulated at a given temperature by the pH of the solution and the time of heating. As shown, for example, in the curve for treatment of the gelatin at pH 10.6, the isoelectric point was reduced after two hours' treatment at 52° C. from 9.17 to 7.04. After five hours' treatment the isoelectric point of this sample had dropped to 6.46 and, after 28 hours' treatment it had dropped to 5.4. As the pH of treatment increased, the rate of decrease in isoelectric point showed an increase. For example, at a pH of treatment of 12.2 the isoelectric point dropped to 5.15 after one hour whereas at a pH of treatment of 10.6 it had dropped only to 7.64 after the same length of time.

In order to illustrate the effect of temperature on the lowering of the isoelectric point of acid-process gelatin, a sample of the same gelatin having an original isoelectric point at pH 9.17 was treated with a sufficient quantity of sodium hydroxide solution to bring the pH of the gelatin to 9.6. At this pH the gelatin was treated at temperatures of from 35° C. to 52° C. and the results recorded as follows:

| Temperature | Time of heating | pH of isoelectric point |      |
|-------------|-----------------|-------------------------|------|
|             |                 | Hours                   |      |
| 35° C.      | 96              |                         | 6.52 |
| 40° C.      | 72              |                         | 5.77 |
| 52° C.      | 50              |                         | 4.91 |

These data are not strictly comparable since the times of heating vary. However, as the temperature was lowered, the time of heating was increased with the hope that the times chosen would decrease the isoelectric point to the same value as that obtained at 52° C. This method was used in an attempt to obtain a gelatin with an isoelectric point at about pH 4.9 to compare with the regular lime-process gelatin whose isoelectric

point is about this pH. In spite of these differences in times of heating the results indicate that the reaction is slowed up by lowering the temperature as was to be expected.

In order to study the effect of variation in the alkali employed, we have used alkali metal hydroxides such as sodium hydroxide, potassium hydroxide and ammonium hydroxide and alkaline earth metal hydroxides such as calcium hydroxide. Results of these tests show that the method employed to raise the pH does not affect the result appreciably.

The swelling of gelatin is one physical property whose minimum range includes the isoelectric point. The swelling of acid-process gelatin is differentiated from that of lime-process gelatins by exhibiting a long pH range of minimum swelling as compared to lime-process gelatin with a sharp minimum at the isoelectric point. Swelling measurements were made on gelatin having an isoelectric point of 6.5 after treatment of an original gelatin having an isoelectric point at pH 8.4. Swelling measurements were made at 15° C. using a sodium acetate-acetic acid buffer and the region of minimum swelling was found to extend from pH 4.5 to pH 10. This indicated that the gelatin had a region of minimum swelling in the same region as that of the isoelectric point.

In using our method for the treatment of lime-process gelatin, we employed a deashed lime-process gelatin having an isoelectric point of 4.78. On heating a sample of this gelatin at 52° C. for five hours at pH 12.2, the isoelectric point decreased slightly from pH 4.78 to pH 4.5. The gelatin thus obtained had been seriously degraded by this treatment which was rather harsh. Aging at pH 12.2 for one month at 5° C. did not decrease the isoelectric point. Under similar conditions the isoelectric point of acid-process gelatin would have been markedly reduced.

This result with lime process gelatin, differing from the result obtained with acid process gelatin is explained by the fact that the hide has lost most of its amide nitrogen during the liming process. Consequently the resulting gelatin has a relatively low isoelectric point and is not affected appreciably by further alkaline treatment.

The use of gelatine of a definite isoelectric point is of value in those cases where standardization of properties, such as swelling, is concerned. In the use of only gelatine of a specific isoelectric point, all external conditions must be regulated by the isoelectric point of the gelatin. If gelatins of all isoelectric points are obtainable then the most desirable conditions with respect to other variables can be selected and a gelatin used whose isoelectric points suit these conditions.

It will be understood that the examples and modifications included herein are illustrative only and that our invention is to be taken as limited only by the scope of the appended claims.

We claim:

1. The method of reducing the isoelectric point of gelatin having an isoelectric point above pH 5, which comprises treating said gelatin at a temperature of from about 30° C. to about 60° C. for a period of time from about 1 minute to about 50 hours with an alkaline hydroxide at a pH greater than about 8, then neutralizing the alkali and washing the gelatin, thereby effecting a reduction in the isoelectric point of the gelatin.

2. The method of reducing the isoelectric point of gelatin having an isoelectric point above pH 5, which comprises treating said gelatin at a tem-

perature of from about 30° C. to about 60° C. for a period of time from about 1 minute to about 50 hours with an alkali metal hydroxide at a pH greater than about 8, then neutralizing the alkali and washing the gelatin, thereby effecting a reduction in the isoelectric point of the gelatin.

3. The method of reducing the isoelectric point of acid-process gelatin, which comprises adding sodium hydroxide to a solution of said gelatin in sufficient amount to bring the pH to about 8, heating the mixture at a temperature of from about 30° C. to about 60° C. for a period of time from about one minute to about 50 hours, neutralizing the alkali with acid, and washing the gelatin with cold water.

4. The method of reducing the isoelectric point of acid-process gelatin, which comprises adding sodium hydroxide to a solution of said gelatin in sufficient amount to bring the pH to about 8, heating the mixture at a temperature of from about 30° C. to about 60° C. for a period of time from about 1 minute to about 50 hours, neutralizing the alkali with hydrochloric acid, and washing the gelatin with cold water.

5. The method of treating gelatin having an isoelectric point above pH 5, to lower the pH of its isoelectric point, which comprises mixing an alkali metal hydroxide with a solution of gelatin at a pH above about 8, heating the mixture at a temperature of approximately 50° C. for a period of time from about one minute to about 50 hours, neutralizing the alkali metal hydroxide with acid, and washing the gelatin with water.

10 6. The method of reducing the isoelectric point of gelatin having an isoelectric point above pH 5, which comprises treating said gelatin with an alkaline material at a temperature of from about 5° C. to about 60° C. at a pH greater than about pH 8 and for a length of time sufficient to effect a reduction in the isoelectric point of the gelatin without appreciably degrading it, then neutralizing the alkaline material and washing the gelatin, thereby effecting a reduction in the isoelectric point of the gelatin.

ROBERT C. HOUCK.  
JOHN RUSSELL.  
SAMUEL E. SHEPPARD.